



US006576186B1

(12) **United States Patent**  
Martin et al.

(10) **Patent No.:** **US 6,576,186 B1**  
(45) **Date of Patent:** **Jun. 10, 2003**

- (54) **ENHANCED MACHINABILITY  
PRECIPITATION-HARDENABLE STAINLESS  
STEEL FOR CRITICAL APPLICATIONS**
- (75) Inventors: **James W. Martin**, Sinking Spring, PA (US); **Roland E. Schmitt**, Mohnton, PA (US); **Ronald C. Gower**, Reading, PA (US)
- (73) Assignee: **CRS Holdings, Inc.**, Wilmington, DE (US)
- (\*) Notice: Subject to any disclaimer, the term of this patent is extended or adjusted under 35 U.S.C. 154(b) by 0 days.

(21) Appl. No.: **09/936,379**

(22) PCT Filed: **Mar. 8, 2000**

(86) PCT No.: **PCT/US00/05916**

§ 371 (c)(1),  
(2), (4) Date: **Nov. 29, 2001**

(87) PCT Pub. No.: **WO00/53821**

PCT Pub. Date: **Sep. 14, 2000**

**Related U.S. Application Data**

- (60) Provisional application No. 60/123,230, filed on Mar. 8, 1999.
- (51) **Int. Cl.** <sup>7</sup> **C22C 38/42**; C22C 38/48
- (52) **U.S. Cl.** **420/60**; 420/61; 148/325
- (58) **Field of Search** **148/325; 420/60;**  
**420/61**

(56) **References Cited**

**U.S. PATENT DOCUMENTS**

- 2,850,380 A 9/1958 Clarke  
4,769,213 A 9/1988 Haswell, Jr. et al.

**OTHER PUBLICATIONS**

Aerospace Material Specification No. AMS 5659H, "Steel, Corrosion Resistant Bars, Wire forgings, Rings, and Extrusions", SAE (1995).

*Primary Examiner*—Deborah Yee

(74) *Attorney, Agent, or Firm*—Dann, Dorfman, Herrell and Skillman, P.C.

(57)

**ABSTRACT**

A precipitation-hardenable, martensitic stainless steel alloy is described having the following composition in weight percent.

|         |              |
|---------|--------------|
| C       | 0.030 max.   |
| Mn      | 1.00 max.    |
| Si      | 1.00 max.    |
| P       | 0.030 max.   |
| S       | 0.005–0.015  |
| Cr      | 14.00–15.50  |
| Ni      | 3.50–5.50    |
| Mo      | 1.00 max.    |
| Cu      | 2.50–4.50    |
| Nb + Ta | (5 × C)–0.30 |
| Al      | 0.05 max.    |
| B       | 0.010 max.   |
| N       | 0.030 max.   |

and the balance is essentially iron and the usual impurities. The alloy provides a unique combination of properties in that useful articles made therefrom provide superior machining characteristics relative to known high strength 15Cr-5Ni precipitation-hardenable stainless steel alloys, while meeting the strength, ductility, and hardness requirements specified in AMS 5659 for critical applications.

**19 Claims, No Drawings**

**ENHANCED MACHINABILITY  
PRECIPITATION-HARDENABLE STAINLESS  
STEEL FOR CRITICAL APPLICATIONS**

This application claims the benefit of priority of U.S. 5  
Provisional Application No. 60/123,230, filed Mar. 8, 1999.

**FIELD OF THE INVENTION**

This invention relates to high strength stainless steel 10  
alloys and, in particular, to a precipitation-hardenable, mar-  
tensitic stainless steel alloy having a unique combination of  
strength, ductility, toughness, and machinability.

**BACKGROUND OF THE INVENTION**

Aerospace material specification AMS 5659 describes a 15  
15Cr-5Ni precipitation hardenable, corrosion resistant steel  
alloy for use in critical aerospace components. AMS 5659  
specifies minimum strength and ductility requirements  
which the alloy must meet after various age-hardening heat  
treatments. For example, in the H900 condition (heated at  
about 900 F. (482 C.) for 1 hour and then air cooled), a  
conforming alloy must provide a tensile strength of at least  
190 ksi (1310 MPa) in both the longitudinal and transverse  
directions together with an elongation of at least 10% in the  
longitudinal direction and at least 6% in the transverse  
direction. However, products manufactured to meet that  
specification typically lack the ease of machinability desired  
by component fabricators.

As the alloy specified in AMS 5659 continues to be used 20  
in many structural components for aerospace applications, a  
need has arisen for an alloy that meets all of the mechanical  
requirements of AMS 5659, but which also provides super-  
ior machinability. It is generally known to add certain  
elements such as sulfur, selenium, tellurium, etc. to stainless  
steel alloys in order to improve their machinability. 25  
However, the inclusion of such "free-machining additives",  
without more, will adversely affect the mechanical proper-  
ties of the alloy, such as toughness and ductility, to the point  
where the alloy becomes unsuitable for the critical structural  
components for which it was designed. Consequently, a need  
exists for a precipitation-hardenable martensitic stainless 30  
steel having good ductility, toughness, and notch tensile  
strength to be useful for critical applications and which also  
provides superior machinability compared with alloy com-  
positions currently utilized for fracture-critical components.

**SUMMARY OF THE INVENTION**

The present invention is directed to a precipitation- 35  
hardenable martensitic stainless steel which provides  
mechanical properties (tensile and notch strength, ductility,  
and toughness) that meet the requirements of AMS 5659 and  
which also provides significantly better machinability com-  
pared to the known grades of 15Cr-5Ni precipitation- 40  
hardenable stainless steels. The broad, intermediate, and  
preferred weight percent compositions of the alloy accord-  
ing to this invention are set forth in the following table.

-continued

| Element | Weight percent |                |                |
|---------|----------------|----------------|----------------|
|         | Broad          | Intermediate   | Preferred      |
| Si      | 1.00 max.      | 0.60 max.      | 0.50 max.      |
| P       | 0.030 max.     | 0.030 max.     | 0.025 max.     |
| S       | 0.005-0.015    | 0.005-0.015    | 0.007-0.013    |
| Cr      | 14.00-15.50    | 14.00-15.50    | 14.25-15.25    |
| 10 Ni   | 3.50-5.50      | 3.50-5.50      | 4.00-5.50      |
| Mo      | 1.00 max.      | 0.50 max.      | 0.50 max.      |
| Cu      | 2.50-4.50      | 2.50-4.50      | 3.00-4.00      |
| Nb + Ta | (5 x C) - 0.30 | (5 x C) - 0.25 | (5 x C) - 0.20 |
| Al      | 0.05 max.      | 0.025 max.     | 0.025 max.     |
| B       | 0.010 max.     | 0.005 max.     | 0.005 max.     |
| 15 N    | 0.030 max.     | 0.025 max.     | 0.010-0.025    |
| Fe      | Bal.           | Bal.           | Bal.           |

The foregoing tabulation is provided as a convenient 20  
summary and is not intended thereby to restrict the lower  
and upper values of the ranges of the individual elements for  
use in combination with each other, or to restrict the ranges  
of the elements for use solely in combination with each  
other. Thus, one or more of the ranges can be used with one  
or more of the other ranges for the remaining elements. In  
25 addition, a minimum or maximum for an element of a broad,  
intermediate, or preferred composition can be used with the  
minimum or maximum for the same element in another  
preferred or intermediate composition. Here and throughout  
this specification the term "percent" or the symbol "%" 30  
means percent by weight unless otherwise specified.

**DETAILED DESCRIPTION OF THE  
INVENTION**

The interstitial elements carbon and nitrogen are restricted 35  
35 to low levels in this alloy in order to benefit the machin-  
ability of the alloy. Therefore, the alloy contains not more  
than about 0.030% each of carbon and nitrogen and prefer-  
ably not more than about 0.025% of each of those elements.  
Carbon and nitrogen are strong austenite stabilizing ele- 40  
ments and limiting them to levels that are too low leads to  
the formation of undesirable amounts of ferrite in this alloy.  
Therefore, at least about 0.010% each of carbon and nitro-  
gen is preferably present in the alloy.

This alloy contains a controlled amount of sulfur to 45  
benefit the machinability of the alloy without adversely  
affecting the ductility, toughness, and notch tensile strength  
of the alloy. To that end, the alloy contains at least about  
0.005% and preferably at least about 0.007% sulfur. Too  
50 much sulfur adversely affects the ductility, toughness, and  
notch tensile strength of this alloy. Therefore, sulfur is  
restricted to not more than about 0.015% and preferably to  
not more than about 0.013% in this alloy.

At least about 14.00% and preferably at least about 55  
14.25% chromium is present in the alloy to provide an  
adequate level of corrosion resistance. However, when chro-  
mium is present in excess of about 15.50% the formation of  
undesirable ferrite results. Therefore, chromium is restricted  
to not more than about 15.50% and preferably to not more  
60 than about 15.25% in this alloy.

At least about 3.50%, preferably at least about 4.00%, 65  
nickel is present in the alloy to maintain good toughness and  
ductility. Nickel also benefits the austenite phase stability of  
this alloy at the low levels of carbon and nitrogen used in the  
alloy. The strength capability of the alloy in the aged  
condition is adversely affected when more than about 5.50%  
nickel is present because of incomplete austenite-to-

| Element | Weight percent |              |             |
|---------|----------------|--------------|-------------|
|         | Broad          | Intermediate | Preferred   |
| C       | 0.030 max.     | 0.025 max.   | 0.010-0.025 |
| Mn      | 1.00 max.      | 0.50 max.    | 0.50 max.   |

martensite transformation (i.e., retained austenite) at room temperature. Therefore, this alloy contains not more than about 5.50% nickel.

At least about 2.50%, preferably at least about 3.00%, copper is present in this alloy as the primary precipitation hardening agent. During the age hardening heat treatment, the alloy achieves substantial strengthening through the precipitation of fine, copper-rich particles from the martensitic matrix. Copper is present in this alloy in amounts ranging from 2.50 to 4.50% to provide the desired precipitation hardening response. Too much copper adversely affects the austenite phase stability of this alloy and can lead to formation of excessive austenite in the alloy after the age hardening heat treatment. Therefore, copper is restricted to not more than about 4.50% and preferably to not more than about 4.00% in this alloy.

A small amount of molybdenum is effective to benefit the corrosion resistance and toughness of this alloy. The minimum effective amount can be readily determined by those skilled in the art. Too much molybdenum increases the potential for ferrite formation in this alloy and can adversely affect the alloy's phase stability by promoting retained austenite. Therefore, while this alloy may contain up to about 1.00% molybdenum, it preferably contains not more than about 0.50% molybdenum.

A small amount of niobium is present in this alloy primarily as a stabilizing agent against the formation of chromium carbonitrides which are deleterious to corrosion resistance. To that end the alloy contains niobium in an amount equivalent to at least about five times the amount of carbon in the alloy (5%C). Too much niobium, particularly at the low carbon and nitrogen levels present in this alloy, causes excessive formation of niobium carbides, niobium nitrides, and/or niobium carbonitrides and adversely affects the good machinability provided by this alloy. Too many niobium carbonitrides also adversely affect the alloy's toughness. Furthermore, excessive niobium results in the formation of an undesirable amount of ferrite in this alloy. Therefore, niobium is restricted to not more than about 0.30%, better yet to not more than about 0.25%, and preferably to not more than about 0.20%. Those skilled in the art will recognize that tantalum may be substituted for

aluminum oxides which are detrimental to the good machinability provided by the alloy. Other elements such as manganese, silicon, and phosphorus are also maintained at low levels because they adversely affect the good toughness provided by this alloy. The composition of this alloy is balanced so that the microstructure of the steel undergoes substantially complete transformation from austenite to martensite during cooling from the annealing temperature to room temperature. As described above, the constituent elements are balanced within their respective weight percent ranges such that the alloy contains not more than about 2 volume percent (vol. %) ferrite, preferably not more than about 1 vol % ferrite, in the annealed condition.

The alloy according to this invention is preferably melted by vacuum induction melting (VIM), but can also be arc-melted in air (ARC). The alloy is refined by vacuum arc remelting (VAR) or electroslag remelting (ESR). The alloy may be produced in various product forms including billet, bar, rod, and wire. The alloy may also be used to fabricate a variety of machined, corrosion resistant parts that require high strength and good toughness. Among such end products are valve parts, fittings, fasteners, shafts, gears, combustion engine parts, components for chemical processing equipment and paper mill equipment, and components for aircraft and nuclear reactors.

The unique combination of properties provided by the alloy according to the present invention will be appreciated better in the light of the following examples.

## EXAMPLES

In order to demonstrate the unique combination of properties provided by the alloy according to the present invention, examples of the alloy were prepared and tested relative to comparative alloys.

### Example 1

Four heats, each weighing approximately 400-pounds, were vacuum-induction melted and cast as single 7.5"-square ingots. The chemical analyses of the heats are shown in Table I in weight percent. Heat 1 is an example of the steel according to this invention. Heats A, B, and C are comparative alloys.

TABLE I

| Heat No. | Element (weight percent) |     |     |      |       |       |      |     |      |     |      |        |      |      |  |
|----------|--------------------------|-----|-----|------|-------|-------|------|-----|------|-----|------|--------|------|------|--|
|          | C                        | Mn  | Si  | P    | S     | Cr    | Ni   | Mo  | Cu   | Nb  | Ta   | B      | N    | Fe   |  |
| 1        | .020                     | .30 | .42 | .021 | .009  | 14.87 | 4.72 | .10 | 3.30 | .15 | <.01 | <.0010 | .017 | Bal. |  |
| A        | .020                     | .30 | .40 | .021 | <.001 | 14.87 | 4.70 | .10 | 3.30 | .15 | <.01 | <.0010 | .017 | Bal. |  |
| B        | .036                     | .31 | .41 | .021 | <.001 | 15.11 | 4.59 | .10 | 3.30 | .26 | <.01 | <.0010 | .017 | Bal. |  |
| C        | .035                     | .30 | .41 | .021 | .009  | 15.13 | 4.66 | .10 | 3.31 | .26 | <.01 | <.0010 | .017 | Bal. |  |

some of the niobium on a weight percent basis. However, tantalum is preferably restricted to not more than about 0.05% in this alloy.

A small but effective amount of boron may be present in amounts up to about 0.010%, preferably up to about 0.005%, to benefit the hot workability of this alloy.

The balance of the alloy composition is iron except for the usual impurities found in commercial grades of precipitation hardening stainless steels intended for similar use or service. For example, aluminum is restricted to not more than about 0.05% and preferably to not more than about 0.025% in this alloy because aluminum can form aluminum nitrides and

55 The ingots were press-forged to 4" square billets, cogged to a 2.125" diam. round bars, and then hot rolled to 0.6875" diam. bar. All the bars were solution annealed by heating them to a temperature of 1040 C., soaking for one hour at that temperature, and then water quenching to room temperature. Further processing consisted of straightening the annealed bars, turning to 0.637" diam., straightening, rough grinding to 0.627" diam., and then grinding the bars to a finish diameter of 0.625".

60 The microstructure and mechanical properties of the bar products were evaluated and compared relative to the requirements of AMS 5659. Table II shows that little or no

ferrite was present in the microstructures of the solution-annealed 0.625" diam. bars.

TABLE II

| (FERRITE CONTENT IN ANNEALED BARS) |                                      | 5 |
|------------------------------------|--------------------------------------|---|
| Heat No.                           | Ferrite Content<br>(Volume Percent)* |   |
| 1                                  | 0.09                                 |   |
| A                                  | None Detected                        |   |
| B                                  | None Detected                        |   |
| C                                  | 0.08                                 |   |
| AMS 5659                           | 2 Maximum                            |   |

\*Measured from tint-etched longitudinal metallographic specimens via image analysis of 100 fields at 1050x screen magnification.

A comparison of room-temperature smooth tensile properties and hardness of the four alloys in the annealed condition is given in Table III. The data presented in Table III includes the 0.2% offset yield strength (0.2% Y.S.) and ultimate tensile strength (UTS) in ksi (MPa), the percent elongation in 4 diameters (% Elong.), the reduction in area (% RA), and the Rockwell C hardness (HRC).

TABLE III

| (LONGITUDINAL SMOOTH TENSILE PROPERTIES AND HARDNESS OF ANNEALED BARS) |              |          |             |         |                          |
|------------------------------------------------------------------------|--------------|----------|-------------|---------|--------------------------|
| Smooth Tensile Properties <sup>(1)</sup>                               |              |          |             |         |                          |
| Heat No.                                                               | .2%<br>Y. S. | UTS      | %<br>Elong. | %<br>RA | HRC <sup>(2)</sup>       |
| 1                                                                      | 135.0        | 149.6    | 15.9        | 70.8    | 31                       |
| A                                                                      | 139.1        | 149.5    | 16.3        | 77.5    | 31                       |
| B                                                                      | 143.6        | 155.3    | 15.8        | 73.9    | 32                       |
| C                                                                      | 138.6        | 154.0    | 15.5        | 70.8    | 32.5                     |
| AMS 5659                                                               | —            | 175 max. | —           | —       | 39.1 max. <sup>(3)</sup> |

<sup>(1)</sup>Average of duplicate specimens.

<sup>(2)</sup>Average of four measurements taken at midradius location.

<sup>(3)</sup>Converted from HB scale.

A comparison of room-temperature smooth tensile properties and hardness was also developed for the alloys in the various aged conditions specified in AMS 5659. Results are presented in Table IV including the 0.2% offset yield strength (0.2% Y.S.) and ultimate tensile strength (UTS) in ksi (MPa), the percent elongation in 4 diameters (Elong.), the reduction in area (RA), and the Rockwell C hardness (HRC).

TABLE IV

| (LONGITUDINAL SMOOTH TENSILE PROPERTIES AND HARDNESS OF AGED-HARDENED BARS) |                          |        |       |         |         |                                        |
|-----------------------------------------------------------------------------|--------------------------|--------|-------|---------|---------|----------------------------------------|
| Smooth Tensile Properties <sup>(1)</sup>                                    |                          |        |       |         |         |                                        |
| Heat No.                                                                    | Condition <sup>(2)</sup> | .2% YS | UTS   | Elong.  | RA      | HRC <sup>(3)</sup>                     |
| 1                                                                           | H900                     | 189.8  | 199.0 | 14.1    | 51.4    | 43                                     |
| A                                                                           | H900                     | 192.8  | 198.6 | 14.5    | 56.6    | 43                                     |
| B                                                                           | H900                     | 193.6  | 199.7 | 14.8    | 59.6    | 43                                     |
| C                                                                           | H900                     | 190.6  | 199.3 | 14.4    | 59.7    | 43                                     |
| AMS 5659                                                                    | H900                     | 170    | 190   | 10 min. | 35 min. | 41.8-<br>min. min. 47.1 <sup>(4)</sup> |
|                                                                             |                          |        |       |         |         | 60                                     |
| 1                                                                           | H925                     | 178.7  | 186.7 | 14.4    | 55.6    | 41                                     |
| A                                                                           | H925                     | 178.6  | 185.3 | 14.5    | 55.1    | 41                                     |
| B                                                                           | H925                     | 179.8  | 184.9 | 16.4    | 64.9    | 41                                     |
| C                                                                           | H925                     | 177.6  | 184.9 | 16.7    | 61.6    | 41                                     |
| AMS 5659                                                                    | H925                     | 155    | 170   | 10 min. | 38 min. | 40.4-<br>min. min. 45.7 <sup>(4)</sup> |
|                                                                             |                          |        |       |         |         | 65                                     |

TABLE IV-continued

| (LONGITUDINAL SMOOTH TENSILE PROPERTIES AND HARDNESS OF AGED-HARDENED BARS) |                          |        |       |         |         |                                        |
|-----------------------------------------------------------------------------|--------------------------|--------|-------|---------|---------|----------------------------------------|
| Smooth Tensile Properties <sup>(1)</sup>                                    |                          |        |       |         |         |                                        |
| Heat No.                                                                    | Condition <sup>(2)</sup> | .2% YS | UTS   | Elong.  | RA      | HRC <sup>(3)</sup>                     |
| 1                                                                           | H1025                    | 159.6  | 163.8 | 15.3    | 62.1    | 36                                     |
| A                                                                           | H1025                    | 157.8  | 162.5 | 16.1    | 63.6    | 36                                     |
| B                                                                           | H1025                    | 160.5  | 164.0 | 16.1    | 65.6    | 36                                     |
| C                                                                           | H1025                    | 159.6  | 163.3 | 16.1    | 65.4    | 36                                     |
| AMS 5659                                                                    | H1025                    | 145    | 155   | 12 min. | 45 min. | 35.5-<br>min. min. 43.1 <sup>(4)</sup> |
| 1                                                                           | H1150                    | 115.3  | 139.0 | 21.3    | 68.9    | 30                                     |
| A                                                                           | H1150                    | 115.8  | 138.6 | 23.3    | 73.2    | 30                                     |
| B                                                                           | H1150                    | 113.3  | 138.2 | 21.7    | 71.7    | 30                                     |
| C                                                                           | H1150                    | 109.6  | 138.1 | 21.8    | 70.2    | 30                                     |
| AMS 5659                                                                    | H1150                    | 105    | 135   | 16 min. | 50 min. | 28.8-<br>min. min. 37.9 <sup>(4)</sup> |

<sup>(1)</sup>Average of duplicate specimens.

<sup>(2)</sup>Aging cycles are defined as follows: H900: 900 F/1 hour/air cool H925: 925 F/4 hours/air cool H1025: 1025 F/4 hours/air cool H1150: 1150 F/4 hours/air cool

<sup>(3)</sup>Average of four measurements.

<sup>(4)</sup>Converted from HB scale.

25 The data presented in Tables III and IV show that the hardness and smooth tensile properties of the four alloys are similar and that they all satisfy the requirements of AMS 5659 under the respective heat treating conditions.

30 The machinabilities of the annealed 0.625" diam. bars of each alloy were tested by employing a Brown and Sharpe Ultramatic (single spindle) Screw Machine. Spindle speed was utilized as the variable test parameter. Three tests were 35 conducted on all four heats at speeds of 95.5 and 104.3 surface feet per minute (SFM). A given trial was terminated for one of two reasons a) part growth exceeding 0.003" as a result of tool wear (Part Growth) or b) at least 400 parts were machined without 0.003" part growth (Discontinued). Cata- 40 strophic tool failure, a third reason for test termination, was not experienced in this testing. The screw machine test parameters and results are provided in Table V, including the spindle speed (Spindle Speed) in SFM, the number of parts machined (Total Parts) and the reason for terminating each 45 test (Reason for Test Termination).

TABLE V

| (SCREW MACHINE TEST RESULTS FOR ANNEALED BARS) |               |             |                             |
|------------------------------------------------|---------------|-------------|-----------------------------|
| Heat No.                                       | Spindle Speed | Total Parts | Reason for Test Termination |
| 1                                              | 95.5          | 400         | Discontinued                |
| 1                                              | 95.5          | 400         | Discontinued                |
| 1                                              | 95.5          | 370         | Part Growth                 |
| 1                                              | 104.3         | 240         | Part Growth                 |
| 1                                              | 104.3         | 180         | Part Growth                 |
| 1                                              | 104.3         | 230         | Part Growth                 |
| A                                              | 95.5          | 110         | Part Growth                 |
| A                                              | 95.5          | 110         | Part Growth                 |
| A                                              | 95.5          | 160         | Part Growth                 |
| A                                              | 104.3         | 90          | Part Growth                 |
| A                                              | 104.3         | 80          | Part Growth                 |
| A                                              | 104.3         | 80          | Part Growth                 |
| B                                              | 95.5          | 40          | Part Growth                 |
| B                                              | 95.5          | 30          | Part Growth                 |
| B                                              | 95.5          | 30          | Part Growth                 |
| B                                              | 104.3         | 30          | Part Growth                 |
| B                                              | 104.3         | 40          | Part Growth                 |

TABLE V-continued

| (SCREW MACHINE TEST RESULTS FOR ANNEALED BARS) |               |             |                             |
|------------------------------------------------|---------------|-------------|-----------------------------|
| Heat No.                                       | Spindle Speed | Total Parts | Reason for Test Termination |
| B                                              | 104.3         | 45          | Part Growth                 |
| C                                              | 95.5          | 90          | Part Growth                 |
| C                                              | 95.5          | 90          | Part Growth                 |
| C                                              | 95.5          | 80          | Part Growth                 |
| C                                              | 104.3         | 50          | Part Growth                 |
| C                                              | 104.3         | 60          | Part Growth                 |
| C                                              | 104.3         | 60          | Part Growth                 |

<sup>(1)</sup>A rough form tool feed rate of 0.002 ipr (inches per revolution) was utilized for all tests.

Set forth in Table VI is a summary of the data presented in Table V above, including the number of parts machined at each spindle speed (Parts Machined). The mean and standard deviation values for the comparative alloys are also shown.

TABLE VI

| (SCREW MACHINE TEST RESULT SUMMARY ANNEALED BARS) |                   |                    |      |
|---------------------------------------------------|-------------------|--------------------|------|
| Heat No.                                          | Mean              | Standard Deviation |      |
| Parts Machines at 95.5 SFM                        |                   |                    |      |
| 1                                                 | >400*, >400*, 370 | —                  | —    |
| A                                                 | 110, 110, 160     | 127                | 28.9 |
| B                                                 | 40, 30, 30        | 33                 | 5.8  |
| C                                                 | 90, 90, 80        | 87                 | 5.8  |
| Parts Machines at 104.3 SFM                       |                   |                    |      |
| 1                                                 | 240, 180, 230     | 217                | 32.1 |
| A                                                 | 90, 80, 80        | 83                 | 5.8  |
| B                                                 | 30, 40, 45        | 38                 | 7.6  |
| C                                                 | 50, 60, 60        | 57                 | 5.8  |

\*Test discontinued because of runout.

When viewed together, the data in Tables II to VI show that Heat 1 provides a significantly better combination of properties relative to Heats A, B, and C, because it provides superior machinability while maintaining the mechanical and microstructural property requirements of AMS 5659.

### Example 2

Six 400 lb. heats were vacuum induction melted and cast as 7½" ingots. The chemical analyses of the heats are shown in Table VII in weight percent. Heats 2, 3, and 4 are examples of the steel according to this invention and Heats D, E, and F are comparative alloys.

TABLE VII

| Heat No. | Element (weight percent) |     |     |      |      |       |      |     |      |     |      |        |      |      |
|----------|--------------------------|-----|-----|------|------|-------|------|-----|------|-----|------|--------|------|------|
|          | C                        | Mn  | Si  | P    | S    | Cr    | Ni   | Mo  | Cu   | Nb  | Ta   | B      | N    | Fe   |
| 2        | .022                     | .45 | .23 | .026 | .006 | 15.31 | 4.73 | .25 | 3.78 | .21 | <.01 | <.0010 | .017 | Bal. |
| 3        | .026                     | .51 | .48 | .023 | .014 | 15.32 | 4.28 | .12 | 3.28 | .20 | <.01 | .0011  | .018 | Bal. |
| 4        | .020                     | .51 | .45 | .028 | .011 | 15.28 | 4.80 | .27 | 3.16 | .20 | <.01 | .0020  | .013 | Bal. |
| D        | .022                     | .44 | .23 | .028 | .003 | 15.29 | 4.73 | .25 | 3.79 | .45 | <.01 | <.0010 | .017 | Bal. |
| E        | .034                     | .63 | .49 | .025 | .020 | 15.71 | 4.29 | .12 | 3.29 | .26 | <.01 | .0011  | .017 | Bal. |
| F        | .020                     | .52 | .45 | .026 | .018 | 15.56 | 4.81 | .27 | 3.16 | .22 | <.01 | .0021  | .013 | Bal. |

Heat 2 was prepared for comparison with Heat D, Heat 3 was prepared for comparison with Heat E, and Heat 4 was prepared for comparison with Heat F. The ingots were press forged to 4" square bars as described above in Example 1.

<sup>5</sup> The 4" square bars of Heats 2 and D were further processed to 5/8" diam. round bars as described above in Example 1.

A comparison of the room-temperature, longitudinal smooth tensile properties and hardness of Heats 2 and D in the annealed and H1150 conditions is given in Tables VIIIA and VIIIB. Prior to testing, the bars of each heat were annealed at 1040 C. for 1 hour and then water quenched. Subsequently, the bars of each heat were age hardened by heating at 1150 F. for 4 hours and then air cooled. The data presented in Tables VIIIA and VIIIB include the 0.2% offset yield strength (0.2% Y.S.) and ultimate tensile strength (UTS) in ksi (MPa), the percent elongation in 4 diameters (% Elong.), the reduction in area (% RA), and the Rockwell C hardness (HRC). Also shown for reference are the tensile and hardness requirements specified in AMS 5659.

TABLE VIIIA

| (SMOOTH TENSILE PROPERTIES AND HARDNESS OF ANNEALED BARS) |           |          |          |      |                    |
|-----------------------------------------------------------|-----------|----------|----------|------|--------------------|
| Annealed Bar Properties <sup>(1)</sup>                    |           |          |          |      |                    |
| Heat No.                                                  | .2% Y. S. | UTS      | % Elong. | % RA | HRC <sup>(2)</sup> |
| 2                                                         | 143.3     | 148.2    | 15.5     | 70.4 | 31                 |
| D                                                         | 134.1     | 138.5    | 15.7     | 72.8 | 27.5               |
| AMS 5659                                                  | —         | 175 max. | —        | —    | 39.1 max.          |

<sup>(1)</sup>Average of duplicate .250" diam. gage smooth tensile specimens.

<sup>(2)</sup>Average hardness on cross section of bar at midradius.

TABLE VIIIB

| (SMOOTH TENSILE PROPERTIES AND HARDNESS OF H1150 BARS) |           |          |          |         |                    |
|--------------------------------------------------------|-----------|----------|----------|---------|--------------------|
| Age-Harden Bar Properties <sup>(1)</sup>               |           |          |          |         |                    |
| Heat No.                                               | .2% Y. S. | UTS      | % Elong. | % RA    | HRC <sup>(2)</sup> |
| 2                                                      | 111.4     | 138.0    | 22.4     | 69.4    | 29.0               |
| D                                                      | 125.2     | 138.2    | 21.1     | 73.1    | 29.0               |
| AMS 5659                                               | 105 min.  | 135 min. | 16 min.  | 50 min. | 28.8-37.9          |

<sup>(1)</sup>Average of duplicate .250" diam. gage smooth tensile specimens.

<sup>(2)</sup>Average hardness on cross section of bar at midradius.

Set forth in Tables IX and X are the results of machinability testing of the 5/8" bars of Heats 2 and D in the H 1150

age-hardened condition. Table IX shows the results for duplicate tests of each heat on the automatic screw machine as described in Example 1 above, including the relative amounts of C, S, and Nb, in weight percent, and the number of parts machined (Total Parts) until test termination. In each case the spindle speed was 104.3 SFM and the tool feed rate was 0.002 inches per revolution (ipr).

TABLE IX

| Heat No. | SCREW MACHINE TEST RESULTS FOR H1150 AGE-HARDENED BARS |      |      | Reason for Test Termination |             |
|----------|--------------------------------------------------------|------|------|-----------------------------|-------------|
|          | % C                                                    | % S  | % Nb | Total Parts                 |             |
| 2        | .022                                                   | .006 | .21  | 140                         | Part Growth |
|          |                                                        |      |      | 160                         | Part Growth |
| D        | .022                                                   | .003 | .45  | 90                          | Part Growth |
|          |                                                        |      |      | 80                          | Part Growth |

Set forth in Table X below are the results of duplicate tool life tests on each heat, including the relative amounts of C, S, and Nb, in weight percent, the tool failure limit (Tool Failure) expressed in inches (cm) to failure and time to failure (sec.), and the volume of material cut from the test bar (Cut Vol.) in  $\text{in}^3$  ( $\text{cm}^3$ ). In this test, lengths of bars of each heat were turned on a single point lathe employing cutting tool having a T15 high speed steel insert. Accelerated feed and machining speed parameters were selected to produce a catastrophic tool failure. All tests were conducted with a spindle speed of 200 SFM and a tool feed rate of .0132 ipr to achieve a material removal rate of 1.78  $\text{in}^3$ /minute.

TABLE X

| Heat No. | TOOL LIFE TEST RESULTS FOR H1150 AGE-HARDENED BARS |      |      | Tool Failure |      |          |
|----------|----------------------------------------------------|------|------|--------------|------|----------|
|          | % C                                                | % S  | % Nb | Inches       | Sec. | Cut Vol. |
| 2        | .022                                               | .006 | .21  | 2.12         | 7.9  | .235     |
|          |                                                    |      |      | 2.23         | 8.3  | .246     |
| D        | .022                                               | .003 | .45  | Avg. 2.18    | 8.1  | .241     |
|          |                                                    |      |      | 1.99         | 7.4  | .220     |
|          |                                                    |      |      | 1.40         | 5.2  | .154     |
|          |                                                    |      |      | Avg. 1.70    | 6.3  | .187     |

The data in Tables IX and X show that Heat 2, representing an alloy according to present invention, provides superior machinability relative to Heat D when the alloys are in the age-hardened condition (H1150).

Set forth in Tables XIA and XIB are the results of smooth and notch tensile, impact toughness, hardness, and fracture toughness testing of the 4" bars of Heats 3, 4, E, and F in the H1150 age-hardened condition. Table XIA presents data for longitudinally oriented specimens and Table XIB presents data for transversely oriented specimens. The results shown in Tables XIA and XIB include the 0.2% offset yield strength (0.2% Y.S.) and ultimate tensile strength (UTS) in ksi (MPa), the percent elongation in 4 diameters (% Elong.), the reduction in area (% RA), the notched tensile strength (NTS) in ksi (MPa), the NTS/UTS ratio (NTS/UTS), the Charpy V-notch impact strength (CVN) in ft-lbs (J), the Rockwell C hardness (HRC), and the fracture toughness ( $K_Q$ ) in ksi $\sqrt{\text{in}}$  (MPa $\sqrt{\text{m}}$ ).

TABLE XIA

| Heat No. | LONGITUDINAL MECHANICAL PROPERTIES OF H1150 AGE-HARDENED BARS |          |         |         |       |      |             |       |
|----------|---------------------------------------------------------------|----------|---------|---------|-------|------|-------------|-------|
|          | Smooth Tensile Properties <sup>(1)</sup>                      |          |         |         |       |      |             |       |
| 3        | 126.0                                                         | 141.7    | 20.8    | 68.6    | 219.5 |      | 106,104,103 | 147.2 |
|          | 127.4                                                         | 142.2    | 21.1    | 68.7    | 222.2 | 1.56 | Avg. 104    | 31    |
| E        | 117.8                                                         | 140.9    | 21.0    | 66.6    | 218.7 |      | 96,94,87    | 123.4 |
|          | 117.1                                                         | 140.6    | 20.9    | 66.5    | 217.1 | 1.55 | Avg. 92     | 31    |
| 4        | 109.4                                                         | 136.5    | 23.4    | 69.7    | 212.2 |      | 140,132,130 | 98.2  |
|          | 110.5                                                         | 137.0    | 23.4    | 71.5    | 212.3 | 1.55 | Avg. 134    | 29    |
| F        | 110.0                                                         | 138.4    | 22.9    | 71.5    | 219.0 |      | 119,117,117 | 92.3  |
|          | 111.7                                                         | 138.5    | 22.4    | 71.2    | 216.6 | 1.57 | Avg. 118    | 29    |
| AMS 5659 | 105 min.                                                      | 135 min. | 16 min. | 50 min. |       |      | 28.8-37.9   | 90.3  |

<sup>(1)</sup>.250" diam. gage smooth tensile specimens.

<sup>(2)</sup> $K_Q = 10$  ( $d = .252"$ ,  $D = .357"$  with root radius of .0010").

<sup>(3)</sup>Average NTS/ Average UTS.

<sup>(4)</sup>Std CVN impact specimens having L-T notch orientation.

<sup>(5)</sup>Average hardness measured on section of fractured CVN impact specimens.

<sup>(6)</sup>Std 1-1/2" thick compact tension specimens having an L-T slot orientation.

TABLE XIB

| (TRANSVERSE MECHANICAL PROPERTIES<br>OF H1150 AGE-HARDENED BARS) |          |          |          |         |                    |                        |                    |                    |
|------------------------------------------------------------------|----------|----------|----------|---------|--------------------|------------------------|--------------------|--------------------|
| Smooth Tensile Properties <sup>(1)</sup>                         |          |          |          |         |                    |                        |                    |                    |
| Heat No.                                                         | *2% Y.S. | UTS      | % Elong. | % RA    | NTS <sup>(2)</sup> | NTS/UTS <sup>(3)</sup> | CVN <sup>(4)</sup> | HRC <sup>(5)</sup> |
| 3                                                                | 125.1    | 141.1    | 17.5     | 53.7    | 218.3              |                        | 51, 46, 45         | 109.0              |
|                                                                  | 123.3    | 140.5    | 18.7     | 59.4    | 220.7              | 1.56                   | Avg. 47            | 108.0              |
| E                                                                | 120.0    | 141.1    | 16.1     | 42.5    | 212.6              |                        | 39, 39, 27         | 106.3              |
|                                                                  | 111.9    | 139.2    | 19.0     | 56.7    | 212.0              | 1.51                   | Avg. 35            | 89.0               |
| D                                                                | 108.6    | 136.8    | 21.1     | 65.0    | 210.0              |                        | 85, 72, 69         | 96.7               |
|                                                                  | 108.4    | 136.0    | 21.0     | 66.0    | 206.9              | 1.53                   | Avg. 75            | 97.8               |
| F                                                                | 110.3    | 138.6    | 19.8     | 58.9    | 208.0              |                        | 55, 55, 50         | 94.0               |
|                                                                  | 108.7    | 138.1    | 19.8     | 58.2    | 206.8              | 1.50                   | Avg. 53            | 29.5               |
| AMS 5659                                                         | 105 min. | 135 min. | 11 min.  | 35 min. |                    |                        | 28.8-37.9          | 85.3               |

<sup>(1)</sup>250" diam. gage smooth tensile specimens.<sup>(2)</sup>K<sub>Q</sub> = 10 (d = .252", D = .357" with root radius of .0010").<sup>(3)</sup>Average NTS/ Average UTS.<sup>(4)</sup>Std CVN impact specimens having T-L notch orientation.<sup>(5)</sup>Average hardness measured on section of fractured CVN impact specimens.<sup>(6)</sup>Std 1-1/2" thick compact tension specimens having an T-L slot orientation.

The data in Table XIA show that Heats 4 and 5, which are alloys according to the present invention, although providing similar smooth and notch tensile properties and hardness relative to Heats E and F, respectively, provide superior impact toughness and fracture toughness characteristics relative to those alloys. Similar results are demonstrated in Table XIB for the transversely oriented specimens, although at somewhat lower levels than the corresponding longitudinal properties. Good impact toughness and fracture toughness are especially important for materials used in critical structural components.

Considering the data presented in Tables VIIIA, VIIIB, IX, X, XIA, and XIB together, they clearly show the superior combination of strength, toughness, ductility, and machinability provided by the alloy according to the present invention.

The terms and expressions which have been employed herein are used as terms of description, not of limitation. There is no intention in the use of such terms and expressions of excluding any equivalents of the elements or features shown and described or portions thereof. However, it is recognized that various modifications are possible within the scope of the invention claimed.

What is claimed is:

1. A precipitation-hardenable, martensitic stainless steel alloy, consisting essentially of, in weight percent, about

|         |              |
|---------|--------------|
| C       | 0.030 max.   |
| Mn      | 0.50 max.    |
| Si      | 1.00 max.    |
| P       | 0.025 max.   |
| S       | 0.007-0.015  |
| Cr      | 14.00-15.50  |
| Ni      | 3.50-5.50    |
| Mo      | 1.00 max.    |
| Cu      | 2.50-4.50    |
| Nb + Ta | (5 x C)-0.25 |
| Al      | 0.05 max.    |
| B       | 0.010 max.   |
| N       | 0.030 max.   |

and the balance is essentially iron and the usual impurities.

2. A precipitation-hardenable, martensitic stainless steel alloy as set forth in claim 1 containing at least about 0.010% carbon.

25 3. A precipitation-hardenable, martensitic stainless steel alloy as set forth in claim 1 containing not more than about 0.013% sulfur.

4. A precipitation-hardenable, martensitic stainless steel alloy as set forth in claim 1 containing at least about 4.00% nickel.

5. A precipitation-hardenable, martensitic stainless steel alloy as set forth in claim 1 containing not more than about 0.50% molybdenum.

30 6. A precipitation-hardenable, martensitic stainless steel alloy as set forth in claim 1 containing not more than about 0.025 nitrogen.

35 7. A precipitation-hardenable, martensitic stainless steel alloy as set forth in claim 1 containing not more than about 4.00% copper.

8. A precipitation-hardenable, martensitic stainless steel alloy, consisting essentially of, in weight percent, about

|         |              |
|---------|--------------|
| C       | 0.025 max.   |
| Mn      | 0.50 max.    |
| Si      | 0.50 max.    |
| P       | 0.030 max.   |
| S       | 0.007-0.015  |
| Cr      | 14.00-15.50  |
| Ni      | 3.50-5.50    |
| Mo      | 0.50 max.    |
| Cu      | 2.50-4.50    |
| Nb + Ta | (5 x C)-0.25 |
| Al      | 0.025 max.   |
| B       | 0.005 max.   |
| N       | 0.025 max.   |

55 and the balance is essentially iron and the usual impurities.

9. A precipitation-hardenable, martensitic stainless steel alloy as set forth in claim 8 containing at least about 0.010% carbon.

60 10. A precipitation-hardenable, martensitic stainless steel alloy as set forth in claim 8 containing not more than about 0.013% sulfur.

11. A precipitation-hardenable, martensitic stainless steel alloy as set forth in claim 8 containing not more than about 15.25% chromium.

65 12. A precipitation-hardenable, martensitic stainless steel alloy as set forth in claim 8 containing at least about 4.00% nickel.

**13**

**13.** A precipitation-hardenable, martensitic stainless steel alloy as set forth in claim **8** containing not more than about 0.20% niobium-plus-tantalum.

**14.** A precipitation-hardenable, martensitic stainless steel alloy as set forth in claim **8** containing at least about 0.010% nitrogen.

**15.** A precipitation-hardenable, martensitic stainless steel alloy as set forth in claim **8** containing not more than about 4.00% copper.

**16.** A precipitation-hardenable, martensitic stainless steel alloy, consisting essentially of, in weight percent, about

|         |                |    |
|---------|----------------|----|
| C       | 0.010–0.025    | 15 |
| Mn      | 0.50 max.      |    |
| Si      | 0.50 max.      |    |
| P       | 0.025 max.     |    |
| S       | 0.007–0.013    |    |
| Cr      | 14.25–15.25    |    |
| Ni      | 4.00–5.50      |    |
| Mo      | 0.50 max.      |    |
| Cu      | 3.00–4.00      |    |
| Nb + Ta | (5 × C) – 0.20 |    |
| Al      | 0.025 max.     |    |
| B       | 0.005 max.     |    |
| N       | 0.010–0.025    |    |

**17.** A steel article that provides a unique combination of machinability, hardness, strength, ductility, and toughness, in the age-hardened condition, said article being formed of a precipitation-hardenable, martensitic stainless steel alloy consisting essentially of, in weight percent, about:

|         |              |
|---------|--------------|
| C       | 0.030 max.   |
| Mn      | 0.50 max.    |
| Si      | 1.00 max.    |
| P       | 0.030 max.   |
| S       | 0.007–0.015  |
| Cr      | 14.00–15.50  |
| Ni      | 3.50–5.50    |
| Mo      | 1.00 max.    |
| Cu      | 2.50–4.50    |
| Nb + Ta | (5 × C)–0.25 |
| Al      | 0.05 max.    |
| B       | 0.010 max.   |
| N       | 0.030 max.   |

and the balance is essentially iron and the usual impurities.

**18.** A steel article as set forth in claim **17** wherein the alloy contains not more than about 0.020% carbon.

**19.** A steel article as set forth in claim **18** wherein the alloy contains not more than about 0.20% niobium+tantalum.

and the balance is essentially iron and the usual impurities.

\* \* \* \* \*